

# UNITED STATES PATENT OFFICE.

TOM COBB KING, OF NEW YORK, N. Y., ASSIGNOR TO NATIONAL METALLURGIC COMPANY, OF JERSEY CITY, NEW JERSEY, A CORPORATION OF NEW JERSEY.

## PROCESS OF PREVENTING THE FORMATION OF SCAFFOLDS IN KILNS.

No. 810,059.

Specification of Letters Patent.

Patented Jan. 16, 1906.

Application filed September 5, 1905. Serial No. 277,114.

*To all whom it may concern:*

Be it known that I, TOM COBB KING, a citizen of the United States, residing at New York, in the county of New York and State of New York, have discovered or invented a new and useful Improvement in Methods of Preventing the Formation of Scaffolds in Kilns, of which improvement the following is a description.

10 My invention relates to method or means for removing masses of fused material which adhere around and to the sides of kilns or retorts used in sintering or agglomerating finely-divided metalliferous bodies. It has been found in the practical use of kilns usually employed for this purpose—viz., long cylindrical retorts lined with refractory substance adapted to be rotated and in which varying temperatures are obtained—that the 15 fused material has a tendency to adhere to the sides of the retort at some point, usually near the point where the highest degree of temperature is attained, and that it is difficult to remove the same when formed.

20 The object of the present invention is to provide a method or means for the easy and speedy removal of such formation without interfering with or stopping the operation of the kiln. I accomplish this purpose by means 25 of a suitable chemical agent—as, for instance calcium fluorid—which is applied at the point where such formation or scaffold occurs and acting as a flux at the temperature attained in the furnace fuses the material and removes 30 said scaffold from the sides of the kiln. In carrying out my method I preferably use a kiln or retort provided with a plurality of blowpipes, one of which I use to bring the material to the proper fusing or partially-fusing température, and the other blowpipe I use to charge calcium fluorid against the material which adheres to and around the sides of the kiln and forms scaffolds for the purpose of fusing and thus removing the same.

35 I have found in practice that ore low in silica forms few rings or scaffolds and that, on the contrary, ores high in silica invariably

form rings or scaffolds, and as the preponderance of all metalliferous-bearing materials have more or less silica the formation of scaffolds during the treatment of the ore in kilns of the character specified is unavoidable, and the removal thereof is a matter of vital importance in the operation of such kilns. Calcium fluorid has the greatest known affinity for silica, and consequently forms a very powerful flux and readily removes the scaffolds when charged against the same. I have found that a kiln producing from one hundred and fifty to two hundred tons of nodules from metalliferous material running about five (5%) per cent. of silica will require about two hundred pounds of calcium fluorid per day, whereas material running about ten (10%) to fifteen (15%) per cent. of silica requires 65 three hundred to five hundred pounds of calcium fluorid per day to remove the scaffolds that form during the operation of the kiln.

I claim as my invention and desire to secure by Letters Patent—

1. The herein-described method for removing scaffolds or rings of fused material from the sides of the kiln which consists in charging against said material, forming such rings or scaffolds, calcium fluorid.

2. The herein-described method of removing adhering masses of material from the sides of kilns or retorts which consists in charging against said material a requisite quantity of calcium fluorid to flux the same.

3. The herein-described method for removing adhering masses of fused material from the sides of the kiln which consists in charging against such adhering masses calcium fluorid and maintaining the material at a high temperature during the charging of said calcium fluorid against the same.

In testimony whereof I have hereunto signed my name in the presence of two subscribing witnesses.

TOM COBB KING.

In presence of—

BENJAMIN A. MORTON,  
GEO. R. A. RICKETTS.